

## UNITED STATES PATENT OFFICE.

JOHN H. MARTIN, OF CENTRAL PARK, NEW YORK.

## CARROTING FUR.

No Drawing.

Application filed December 17, 1924. Serial No. 756,553.

In the carotting of fur hair, that is to say, the preparation of fur hair for felting, particularly for the manufacture of hats, the fur hair or fur, as it will be designated for brevity, either on the skin or after its removal from the skin, is subjected to the action of chemicals which, upon one theory or another, so change the character of the fur and particularly the character of the outer sheath or horny layer, as to promote the interlocking of the fur hairs in the process of shrinking and felting. Whether this change is in the way of freeing scales which interlock or of otherwise changing the character of the outer layer is immaterial, although it is believed that the effect of the practice of the present invention is to bring about a change other than the freeing of scales. As is well understood in the art, the chemical employed, generally in solution, is sometimes brushed into the fur on the skin, the fur being subsequently removed, and is sometimes used as a bath in which are immersed the fur hairs after removal from the skin. In either case the fur is dried after treatment with the chemical and is thereafter subjected to the dyeing and felting processes as may be desired. Various chemicals have been used or proposed to be used heretofore, some of which, like mercuric nitrate, have made the fur poisonous to those who handle it in subsequent processes, while others, such as those which are more or less strongly alkaline, having a free alkali in composition, bring about a progressive weakening of the hair core such that in the process of aging which is generally practiced by a hat maker, the fur deteriorates in quality.

In the investigation of the art and in the development of the present invention, it has been found that the desired oxidation of the fur, which is the characteristic feature of the process of preparation, can be accomplished, without leaving any poisonous or harmful deposit on the fur and without injuring the texture of the fur, while leaving it in favorable condition for subjection to subsequent treatment, such as dyeing, and promoting the union of the fur hairs in the process of shrinking and felting, by treatment of the fur, either on the skin or after its removal from the skin, with a solution of one of the persalts, such, for example, as ammonium persulphate, potassium percarbonate, or sodium perborate. According to

the results desired and to the subsequent treatment, one or another of the persalts might be used by itself or two or more might be used in mixture. The solution of the persalt or persalts is preferably in pure water. If the particular chemical employed is relatively deficient in oxygen, the deficiency can be supplied by the addition of hydrogen peroxide which by itself has been found not to give satisfactory felting qualities. When added to one of the persalts, however, the hydrogen peroxide will assist in carrying the oxidation of the fur hairs to the desired extent.

By the use of persalts, with or without the addition of hydrogen peroxide as may be required, it is possible to avoid that degree of alkalinity, characterized by the presence of free alkali, which makes the solution alkaline and affects injuriously the texture of the fur.

The alkaline quality of the decomposition product of a percarbonate or a perborate, for example, can be corrected by mixing with it, for example, an equimolecular quantity of a persulphate, the decomposition product of which by itself would give an acid reaction.

As indicated, the persalt employed is preferably of the alkali metal group of persalts, such as potassium percarbonate or sodium perborate or of the alkali earth metal group of persalts, such as the persalts of calcium and barium, the choice of the group depending to some extent upon the character of the fur being treated or upon the particular results to be produced.

It will be understood that the mention herein of specific chemicals is by way of example and illustration only, and that the invention, in its broadest aspect, is not limited to the employment of one chemical or another of the broad group referred to.

I claim as my invention:

1. The improvement in the art of carotting fur which consists in subjecting the fur to the action of a solution of a persalt.

2. The improvement in the art of carotting fur which consists in subjecting the fur to the action of a persalt with the addition of hydrogen peroxide.

3. The improvement in the art of carotting fur which consists in subjecting the fur to the action of a solution of a perborate.

4. The improvement in the art of carotting fur which consists in subjecting the fur

to the action of a solution of perborate of sodium.

5. The improvement in the art of carrott-  
ing fur which consists in subjecting the fur

5 to the action of a solution of a perborate with the addition of hydrogen peroxide.

6. The improvement in the art of carrott-

ing fur which consists in subjecting the fur to the action of a solution of perborate of sodium with the addition of hydrogen per- 10  
oxide.

This specification signed this 15th day of December A. D. 1924.

JOHN H. MARTIN.